

## 1

3,245,787  
**PRODUCTION OF COLOR PHOTOGRAPHIC  
 IMAGES**

Jozef Frans Willems, Wilrijk-Antwerp, and Jan Jaeken, Hove-Antwerp, Belgium, assignors to Gevaert Photo-Producten N.V., Mortsel, Belgium, a Belgian company  
 No Drawing. Filed Nov. 14, 1960, Ser. No. 71,117  
 Claims priority, application Great Britain, Nov. 13, 1959,  
 38,551/59  
 12 Claims. (Cl. 96—9)

The present invention relates to the production of colored photographic images, more particularly to a process of color correction utilizing an integral masking procedure.

It is known that dyes formed by color development in subtractive multicolor photographic pictures do not transmit all of the light which theoretical considerations demand. The cyan dye which should absorb red light and transmit green and blue light usually absorbs a small amount of green and blue light, as well as a major proportion of red light. The magenta dye which should absorb green light and transmit blue and red light usually absorbs a considerable amount of blue light and a small amount of red light, as well as a major proportion of green light. The yellow dye which should absorb blue light and transmit green and red light is usually satisfactory.

Due to the above mentioned unwanted side-absorptions of the dyes formed by color development, it is practically impossible to obtain a true reproduction of the original colors on printing multicolor photographic transparencies containing such dyes.

Correction of the colors on printing is therefor desirable, and this is usually done by masking. Since separate masks are difficult to register with the color transparency, it is desirable that the mask be integral with the colored images.

A process for the production of a color photographic image wherein the mask is integral with the colored image is described in U.S. patent applications Ser. No. 705,508, filed December 27, 1957, by Maurice Antoine de Ramaix and Jan Jaeken, now U.S.P. 3,012,884, and Ser. No. 66,944, now U.S. Patent 3,079,256 filed November 3, 1960, by Raphael Karel Van Poucke, Arthur Henri De Cat and Marcel Hendrik Verbrugge for process for the manufacture of photographic color images and color correction, and German patent application G 30,580, filed September 27, 1960, now German Patent 1,119,666.

According to said pending applications a color corrected image is formed in a photographic element comprising a silver halide emulsion layer and a color coupler (more particularly a color coupler of the naphthol type) which is reactive with the oxidation product of an aromatic amino developing agent to form by color development a primary dye image which absorbs a major proportion of light in one region of the visible spectrum (more particularly the red light) and undesirably absorbs a minor proportion of light in at least one other region of the visible spectrum (more particularly the green light), by treating the exposed and color-developed photographic element with an oxidizing solution, more particularly a photographic bleaching bath, in the presence of a compound more particularly a 4-amino-pyrazolone-3-compound, which after oxidation couples with the residual color coupler, whereby a secondary dye image having a gradation opposite to that of said primary dye image, and absorbing light in at least one of said unwanted minor absorption regions (more particularly the green light) but transmitting substantially all

## 2

the light in said major absorption region (more particularly the red light) is formed.

It is an object of the present invention to provide a new method for correcting the colors of a photographic image used for printing. A further object is to provide a new method for the preparation of an integral mask in color film, more particularly to provide a yellow colored mask image compensating the unwanted absorption of blue light by the magenta image dye. Other objects will appear from the following description and examples.

These objects are accomplished by treating an image-wise exposed photographic element comprising a silver halide emulsion layer and a color coupler which is reactive with the oxidation product of an aromatic amino developing agent to form by color development a primary dye image, after the color forming development, with an oxidizing solution, such as a photographic bleaching bath, in the presence of a compound (called hereinafter mask forming compound) containing a grouping of the following structure:



wherein

R<sub>1</sub> represents a hydrogen atom or an acetyl group,  
 R<sub>2</sub> represents a hydrogen atom or a functional substituent which is sufficiently unstable for splitting off during the oxidative coupling, such as e.g. a radical of the formula —SO<sub>2</sub>—X<sub>2</sub> or —CO—X<sub>2</sub> wherein X<sub>2</sub> represents an hydroxyl radical, an amino radical, a substituted amino radical such as a dialkylamino radical, and an N-morpholinyl radical, a hydrocarbon radical or a substituted hydrocarbon radical, such as an alkyl radical e.g. a methyl radical or a cetyl radical, a substituted alkyl radical such as an aralkyl radical and a chloromethyl radical and a carbocyclic radical, e.g. an aryl radical such as e.g. a phenyl radical, and a substituted aryl radical such as e.g. a p-tolyl radical, a 2,5-dichlorophenyl radical and a 2-decanoylamino-phenyl radical, and a heterocyclic radical,

R<sub>3</sub> represents an alkyl radical such as a methyl radical and an ethyl radical, a substituted alkyl radical such as an aralkyl radical and an alkylene radical forming part of a carbocyclic or heterocyclic ring, an aryl radical, a substituted aryl radical, and a radical of the formula —SO<sub>2</sub>—X<sub>3</sub> or —CO—X<sub>3</sub> wherein X<sub>3</sub> represents a hydrocarbon radical such as an alkyl radical, a substituted alkyl radical, and a carbocyclic radical such as an aryl radical, and a heterocyclic radical,

L<sub>1</sub> and L<sub>2</sub> each represents a methine group or a nitrogen atom, at least one of L<sub>1</sub> and L<sub>2</sub> being a methine group, and

n is a positive integer from 1 to 2.

According to a preferred embodiment of our present invention, as mask forming compounds are used: heterocyclic sulphonyl-, respectively acyl-hydrzones of the general formula:



wherein Z represents the non-metallic atoms necessary to complete a heterocyclic nitrogen nucleus such as e.g. a benzothiazole nucleus, a benzoxazole nucleus, a benzimidazole nucleus, a thiazoline nucleus, and a 2-quinoline nucleus, and

R<sub>1</sub> and R<sub>2</sub> have the value as set further hereinbefore.

Heterocyclic sulphonyl and acylhydrzones which can



(25) (26) (27) (28) (29) (30) 

The heterocyclic alkylsulfonylhydrazone mask compounds according to this invention can be prepared e.g. by using one of the following methods.

(1) By condensing a sulfonylchloride compound with an unsubstituted hydrazone.



(2) By reaction of a sulfonylhydrazide with a methyl-mercaptopyclammoniumsalt.



#### PREPARATION 1

##### *N*-ethyl-benzthiazolone-cetyl sulfonhydrazone

38.6 g. (0.2 mol) of *N*-ethylbenzthiazolone hydrazone prepared according to K. Fuchs, Ber. 61, p. 59 (1928), and 32.4 g. (0.1 mol) of cetyl sulfonylchloride are refluxed together for 2 hours with 600 cm<sup>3</sup> of acetonitrile. The formed precipitate of hydrazone-hydrochloride is sucked off when still warm, whereafter the filtrate is cooled. After recrystallization of the resulted crystals

from methanol, 39 g. of *N*-ethyl-benzthiazolone cetyl sulfonhydrazone are obtained. Melting point: 115° C.

#### PREPARATION 2

##### *N*-methyl-quinolone-(2)-cetyl sulfonhydrazone

2.33 g. (0.0075 mol) of 1-methyl-2-methylthio-quinoliniumiodide prepared according to O. Fischer, Ber. 35 p. 3677 (1902), and 2.4 g. (0.0075 mol) of cetyl sulfonylhydrazide are heated for 48 hours at 50° C. with 30 cm<sup>3</sup> 10 pyridine until the evolution of methylmercaptane has ceased. After pouring out the reaction mixture into water, the obtained solid product is washed with water and dried and 2 g. of *N*-methyl-quinolone-(2)-cetyl sulfonhydrazone are obtained. Melting point: 101° C. A recrystallization from acetonitrile increases the melting point up to 110° C.

#### PREPARATION 3

20 *N,N'*-dimethyl-benzimidazolone-cetyl sulfonhydrazone 9 g. (0.03 mol) of 1-3-dimethyl-2-methylthiobenzimidazoliniummethylsulfate prepared by S. Hünig, Ann., 609 p. 107 (1957), and 9.6 g. (0.03 mol) of cetyl sulfonylhydrazide are mixed at room temperature with 75 25 cm<sup>3</sup> of pyridine. After 48 hours the evolution of methylmercaptane has ceased. The reaction mixture is poured into water, the resulting precipitate is washed with water, sucked off and dried. After recrystallization from methanol 5.3 g. of *N,N'*-dimethyl-benzimidazolone-cetyl sulfonhydrazone are obtained. Melting point: 113° C.

#### PREPARATION 4

##### *N*-methyl-benzoxazolone-cetyl sulfonhydrazone

35 8.3 g. (0.05 mol) of 2-methylthio-benzoxazole prepared according to S. Hünig, Ann., 609, p. 169 (1957), and 9.3 g. (0.05 mol) of *p*-tolusulfonic acid methylester are heated for 30 min. at 1500 C. After cooling, the reaction product is washed with ether. 4.2 g. (0.012 mol) of the obtained tolsulfonate are mixed with 3.9 g. 40 (0.012 mol) cetyl sulfonylhydrazide dissolved in 50 cm<sup>3</sup> pyridine. The reaction proceeds at room temperature for 24 hours. After pouring out the reaction mixture into water and washing with water, the obtained product is dried. After recrystallization from methanol the obtained *N*-methyl-benzoxazolone cetyl sulfonhydrazone melts at 98° C.

#### PREPARATION 5

##### *N*-methyl-thiazolinone-cetyl sulfonhydrazone

50 1.38 g. (0.005 mol) of 2-methylthio-3-methyl-thiazoliniumiodide and 1.6 g. (0.005 mol) of cetyl sulfonylhydrazide are mixed and heated for 24 hours at 50° C. with 15 cm<sup>3</sup> of pyridine and 1.5 cm<sup>3</sup> of piperidine. After pouring out into water, the reaction product is washed with water and dried. The hydrazone thus obtained is recrystallized from methanol. 1.7 g. of *N*-methyl-thiazolinone-cetyl sulfonhydrazone are obtained. Melting point: 98° C.

#### PREPARATION 6

##### *N*-ethyl-benzthiazolone-(*m*-decanoylamino-phenyl)-sulfonhydrazone

65 38.6 g. (0.2 mol) of *N*-ethyl-benzthiazolone hydrazone prepared according to K. Fuchs, Ber. 61, p. 59 (1928), 44.3 g. (0.2 mol) of *m*-nitrobenzene sulfochloride and 34 g. (0.4 mol) of anhydrous sodiumacetate are mixed with 600 cm<sup>3</sup> of acetonitrile and refluxed for 2 hours. The reaction mixture is poured out into water. The solid 70 product obtained is washed with water, separated and dried. 62 g. of *N*-ethylbenzthiazolone-(*m*-nitrophenyl)-sulfonhydrazone are obtained. Melting point: 222° C. A recrystallization of acetonitrile does not increase the melting point. 18.9 g. (0.05 mol) of the obtained hydrazone are dissolved in 150 cm<sup>3</sup> of dioxane, 150 cm<sup>3</sup> of

acetic acid and 30 cm.<sup>3</sup> of water. The reduction is carried out at boiling temperature by portion-wise adding 17 g. of iron-filing. After adding, the reaction mixture is further heated for 30 min. Then the reaction mixture is poured out into water, the solid product is washed with water and dried. 16 g. of N-ethyl-benzthiazolone-(m-aminophenyl)-sulfonylhydrazone are obtained. Melting point: 230° C. After recrystallization from acetonitrile, the melting point increases to 238° C. 1.74 g. (0.005 mol) of the above-mentioned aminoderivative and 1 g. (0.0052 mol) of decanoylchloride are heated to boiling in 50 cm.<sup>3</sup> of acetonitrile in such a way that the hydrogen chloride formed distils off simultaneously with a part of acetonitrile. On cooling, 2.2 g. of N-ethyl-benzthiazolone-(m-decanoylamino-phenyl) sulfonylhydrazone crystallizes out. Melting point: 167° C. A further recrystallization from isopropanol does not increase the melting point.

The process of color correction of the present invention may be practiced, i.e., by using a color photographic material containing a coupler for magenta belonging to the class of the pyrazolone or indazolone color couplers and/or a coupler for cyan belonging to the class of the phenol or naphthol color couplers. Depending upon the structure of the color coupler used in combination with the hydrazone mask-forming compound according to the present invention, yellow to magenta colored mask images are obtained on treating the photographic material with an oxidizing substance such as present in a ferricyanide bleaching bath.

According to a preferred embodiment of the present invention, the hydrazone mask forming compound is incorporated in one of the layers present in the light-sensitive photographic material, preferably in the silver halide emulsion layer wherein the mask image is to be formed by oxidative coupling of the residual color coupler present in that layer with the mask forming substance; in order to prevent the diffusion of the mask forming compound out of the silver halide emulsion layer wherein this compound originally was incorporated, preferably heterocyclic sulfonyl or acyl hydrazone mask forming compounds are used containing a radical (e.g. the radical X<sub>2</sub> and/or X<sub>3</sub> in the above formula) comprising a linear chain of 5 to 20 carbon atoms.

For carrying out the process according to the present invention, the color couplers and mask compounds can be incorporated into a photographic silver halide emulsion prepared by means of the colloids usually employed therefor such as for instance gelatin, polyvinyl alcohol, collodion or other natural or synthetic colloids. The silver halide emulsion can be cast to a support consisting of paper, glass, nitrocellulose, cellulose esters such as cellulose triacetate, polyester, polystyrene or another natural or synthetic resin, and form part of a photographic material with one or more emulsion layers. The multilayer material usually comprises the following elements: a support, a red sensitive emulsion layer having a color coupler for cyan, a green sensitive emulsion layer having a color coupler for magenta and a blue sensitive emulsion layer having a color coupler for yellow. Usually there is a yellow filter, composed in most of the cases of colloidal silver, located between the blue-sensitive and the emulsion layer sensitized to green. It is not only possible to incorporate the color couplers into the light-sensitive silver halide emulsion layer itself but they can also be incorporated into an adjacent non-light-sensitive colloid layer or into a non-light-sensitive layer which is separated from the light-sensitive emulsion layer by a water-permeable colloid layer.

The following aromatic amino-compounds can be used as developers for such material: mono-, di- and triamino-aryl compounds, more especially N,N-dialkyl-p-phenylenediamines, such as N,N-diethyl-p-phenylenediamine and N,N-diethyl-2-methyl-p-phenylenediamine, and derivatives

thereof such as N,N-dialkyl-N'-sulphomethyl- or carboxymethyl-p-phenylenediamine. As useful monoamino-developers should be cited: aminophenols and amino-cresols or their halogen derivatives and also the aminonaphthols.

The following examples illustrate the invention without limiting, however, the scope thereof.

#### EXAMPLE 1

To 1/2 kg. of a green-sensitized silver bromo-iodide emulsion containing 1/6 mol of silver halide is added a slightly alkaline alcoholic solution containing 9 g. of 1-p-sulfophenyl-3-heptadecyl-5-pyrazolone and 6 g. of 3-ethyl-2-benzthiazolone-β-cetyl sulphonyl hydrazone of the following formula:



dissolved by heating in alcohol/water (1:3) with a little sodium hydroxide. After acidification with acetic acid to pH 6 and after addition of the usual additives such as hardeners, wetting agents and stabilizers, the emulsion obtained is coated on a suitable support and dried. After exposure through a grey wedge with a constant 0.15, the photographic material is developed for 9 minutes at 20° C. in a color developing bath with the following composition:

|                                              | G.  |
|----------------------------------------------|-----|
| Sodium hexametaphosphate                     | 2   |
| N,N-diethyl-p-phenylenediamine hydrochloride | 3   |
| Sodium sulphite                              | 4   |
| 35 Sodium carbonate                          | 57  |
| Hydroxylamine hydrochloride                  | 1.5 |
| Potassium bromide                            | 1   |
| Water to 1000 cm. <sup>3</sup> (pH=10.6).    |     |

This material is rinsed for 30 minutes at 18 to 20° C. and fixed for 5 minutes at 20° C. in a fixing bath of the following composition:

|                                        | G.  |
|----------------------------------------|-----|
| Sodium thiosulphate                    | 200 |
| Sodium bisulphite                      | 25  |
| Potassium alum                         | 20  |
| Sodium biacetate                       | 20  |
| Boric acid                             | 7.5 |
| Water to 1000 cm. <sup>3</sup> (pH=4). |     |

Next, the material is rinsed again for 10 minutes at 18 to 20° C. and treated for 5 minutes in a bleaching bath of the following composition:

|                                          | G.  |
|------------------------------------------|-----|
| 55 Potassium ferricyanide                | 100 |
| Potassium bromide                        | 15  |
| Borax                                    | 20  |
| Magnesium sulphate                       | 50  |
| Water to 1000 cm. <sup>3</sup> (pH=8.6). |     |

Rinsing is continued for another 10 minutes at 18 to 20° C. and then the material is fixed again for 5 minutes at 20° C. in a bath of the following composition:

|                                          | G.  |
|------------------------------------------|-----|
| 65 Sodium thiosulphate                   | 130 |
| Borax                                    | 20  |
| Magnesium sulphate                       | 50  |
| Water to 1000 cm. <sup>3</sup> (pH=8.9). |     |

Finally, rinsing is continued for 10 minutes at 18 to 20° C. and the material is dried.

A mainly magenta colored image is obtained together with a yellow dye image, said yellow image being of opposite gradation in respect of the magenta dye image and reducing the disturbing influence of the side absorptions in the formed magenta image.

## EXAMPLE 2

To  $\frac{1}{2}$  kg. of a green-sensitized silver bromo-iodide emulsion containing  $\frac{1}{16}$  mol of silver halide is added a slightly alkaline alcoholic solution containing 9 g. of 2-(1-phenyl-5-oxo-3-pyrazolinylimino)-3-carbethoxy-4-[p(1-cetoxy-phenyl)-thiazoline, and 6 g. of 3-ethyl-2-benzthiazolone- $\beta$ -cetyl sulphonyl hydrazone of the following formula:



dissolved by heating in alcohol/water (1:3) with a little sodium hydroxide. After acidification with acetic acid to pH 6 and after addition of the usual additives such as hardeners, wetting agents and stabilizers, the emulsion obtained is ready to be coated. After coating this emulsion forms part of a multilayer photographic material consisting of the following superposed layers in the indicated sequence: a support, an antihalation layer, a gelatin insulating layer, a red-sensitized emulsion layer with color coupler for cyan, a gelatin interlayer, the above-mentioned green-sensitized emulsion layer, a yellow filter layer, a blue-sensitive emulsion layer with color coupler for yellow and at least a gelatin overcoat as antistress layer.

After exposure through a grey wedge with a constant 0.15 the photographic material is developed and further treated as in Example 1.

A mainly magenta colored image is obtained together with a yellow dye image in the green-sensitized layer, said yellow image being of opposite gradation in respect of the magenta dye image and reducing the distributing influence of the side-absorptions in the formed magenta image.

We claim:

1. In a method of forming a color corrected image in a photographic element having at least one silver halide emulsion layer containing a color coupler for magenta which is reactive with the oxidation product of an aromatic amino developing agent to form by color development a magenta primary dye image which absorbs a major proportion of light in one region of the visible spectrum, and undesirably absorbs a minor proportion of light in at least one other region of the visible spectrum, in which method said element is exposed to said image to be photographed, developed with said developing agent and thereafter treated with an oxidizing solution, the improvement which comprises carrying out said development and said treatment in the presence of a mask forming compound having the formula:



wherein:

R1 is a member of the group consisting of a hydrogen atom and an acetyl group,

R2 is a member of the group consisting of an alkyl radical and an aryl radical,

Z represents the non-metallic atoms necessary to complete a heterocyclic nucleus containing 5-6 members, at least one of which is a nitrogen atom, and

X is a member of the group consisting of an hydroxyl radical, an amino radical, an alkyl radical, an aryl radical, and a heterocyclic radical;

whereby the residual color coupler oxidatively couples with said mask-forming compound to form a secondary dye image having a gradation opposite to that of said magenta primary dye image, said secondary image absorbing light in at least one of said undesirable minor ab-

sorption regions but transmitting substantially all the light in said major absorption region.

2. The method of claim 1 wherein said color coupler for magenta is a member of the group consisting of the 5 pyrazolone and indazolone color couplers.
3. The method of claim 1 wherein said mask-forming compound is incorporated in the photographic element and the oxidizing solution is a photographic bleaching bath.
- 10 4. The method of claim 1 wherein said mask-forming compound is present in at least said one layer containing said color coupler.
5. The method of claim 1 wherein said mask-forming compound forms a yellow secondary dye image.
- 15 6. A color photographic element useful in the method of claim 1, said element having superposed silver halide emulsion layers sensitive to different regions of the visible spectrum, at least one of said layers containing a color coupler for magenta which is reactive with the oxidation 20 product of an aromatic amino developing agent to form by color development a magenta primary dye image which absorbs a major proportion of light in one region of the spectrum, and undesirably absorbs a minor proportion of light in at least one other region of the visible spectrum, such layer also containing a mask-forming compound of the formula:



wherein:

R1 is a lower alkyl radical,

Z represents the non-metallic atoms necessary to complete a heterocyclic nitrogen nucleus, and

X is an organic radical comprising a linear chain of 5 to 20 carbon atoms free of ethylenic unsaturation,

said color coupler for magenta also being reactive with the oxidation product of said mask-forming compound to 30 form a secondary dye image having a gradation opposite to that of said magenta primary dye image, and absorbing light in at least one of said unwanted minor absorption regions but transmitting substantially all the light in said major absorption region.

- 40 7. In a method of forming a color corrected image in a photographic element having at least one silver halide emulsion layer containing a color coupler for cyan which is reactive with the oxidation product of an aromatic amino developing agent to form by color development a cyan primary dye image which absorbs a major proportion of light in one region of the visible spectrum, and undesirably absorbs a minor proportion of light in at least one other region of the visible spectrum, in which method 50 said element is exposed to said image to be photographed, developed with said developing agent and thereafter treated with an oxidizing solution, the improvement which comprises carrying out said development and said treatment in the presence of a mask-forming compound having the formula:
- 55 60



wherein:

R1 is a member of the group consisting of a hydrogen atom and an acetyl group,

R2 is a member of the group consisting of an alkyl radical and an aryl radical,

Z represents the non-metallic atoms necessary to complete a heterocyclic nucleus containing 5-6 members, at least one of which is a nitrogen atom, and

X is a member of the group consisting of a hydroxyl

11

radical, an amino radical, an alkyl radical, an aryl radical, and a heterocyclic radical;

whereby the residual color coupler oxidatively couples with said mask-forming compound to form a secondary dye image having a gradation opposite to that of said cyan primary dye image, said secondary image absorbing light in at least one of said undesirable minor absorption regions but transmitting substantially all the light in said major absorption region.

8. The method of claim 7 wherein said color coupler for cyan is a member of the group consisting of the phenol and naphthol color couplers.

9. The method of claim 7 wherein said mask-forming compound is incorporated in the photographic element and the oxidizing solution is a photographic bleaching bath.

10. The method of claim 7 wherein said mask-forming compound is present in at least said one layer containing said color coupler.

11. The method of claim 8 wherein said mask-forming compound forms a magenta secondary dye image.

12. A color photographic element useful in the method of claim 7, said element having superposed silver halide emulsion layers sensitive to different regions of the visible spectrum, at least one of said layers containing a color coupler for cyan which is reactive with the oxidation prod-

uct of an aromatic amino developing agent to form by color development a cyan primary dye image which absorbs a major proportion of light in one region of the spectrum, and undesirably absorbs a minor proportion of light in at least one other region of the visible spectrum, such layer also containing a mask-forming compound of the formula:



wherein:

5

$\text{R}_1$  is a lower alkyl radical,  $\text{Z}$  represents the non-metallic atoms necessary to complete a heterocyclic nitrogen nucleus, and

$\text{X}$  is an organic radical comprising a linear chain of 5 to 20 carbon atoms free of ethylenic unsaturation,

said color coupler for cyan also being reactive with the oxidation product of said mask-forming compound to form a secondary dye image having a gradation opposite to that of said cyan primary dye image, and absorbing light in at least one of said unwanted minor absorption regions but transmitting substantially all the light in said major absorption region.

15

### References Cited by the Examiner

#### UNITED STATES PATENTS

|           |         |                  |         |       |
|-----------|---------|------------------|---------|-------|
| 2,396,396 | 3/1946  | Stammers         | -----   | 96-55 |
| 2,527,476 | 10/1950 | Braylants et al. | -----   | 96-55 |
| 2,895,825 | 7/1959  | Pelz et al.      | -----   | 96-55 |
| 3,012,884 | 12/1961 | De Ramaix et al. | 96-55 X | X     |
| 3,028,237 | 4/1962  | Loffler          | -----   | 96-9  |
| 3,047,385 | 7/1962  | De Ramaix et al. | -----   | 96-9  |

#### FOREIGN PATENTS

|         |         |                |
|---------|---------|----------------|
| 685,061 | 12/1952 | Great Britain. |
| 790,327 | 2/1958  | Great Britain. |

NORMAN G. TORCHIN, Primary Examiner.

HAROLD N. BURSTEIN, Examiner.

R. A. BURROUGHS, J. T. BROWN,  
Primary Examiners.

35